

Aug. 31, 1948.

W. F. REAGER

2,448,496

ANNEALED SHELL

Filed Oct. 22, 1943



William F. Reager

INVENTOR

BY *Thomas E. Mafford*

ATTORNEY

## UNITED STATES PATENT OFFICE

2,448,496

## ANNEALED SHELL

William F. Reager, Tamaqua, Pa., assignor to  
 Atlas Powder Company, Wilmington, Del., a  
 corporation of Delaware

Application October 22, 1943, Serial No. 507,267

3 Claims. (Cl. 102—28)

1

The present application relates to explosion initiators of the bursting type.

An object of the present invention is to provide an improved explosion initiator.

Another object of the invention is to provide an improved squib.

A further object of the present invention is to provide an explosion initiator in which the initiating force is directed in a desired manner.

A still further object of the present invention is to provide an explosion initiator which is easily rupturable.

Still another object of the invention is to provide an explosion initiator in which the initiating force is localized and controlled.

Another object of the invention is to provide an explosion initiator which at the same time is easily rupturable and will tenaciously hold a sealing plug.

Again another object of the present invention is to provide a method for the manufacture of explosion initiators having properties as set forth above.

Other objects of the present invention will be apparent from the following specification.

Explosion initiators usually comprise tubular metal shells containing initiating charges which are designed to burst the shells when providing initiating action. Generally, initiator shells are drawn to the form desired with integral bottom portions against which the explosive charge is loaded, but other methods of working to shape, such as stamping, for example, may be employed.

Prior art explosion initiators have often given difficulty in that the initiating force has not been controlled in direction. This tendency has been particularly noticed in connection with electric squibs which contain a plug seal at the top end. Such plugs have often tended to blow out, permitting the initiating force to escape out the top rather than bursting the shell of the initiator as is usually desired. The present invention will be specifically illustrated in connection with electric squibs.

The drawing shows a view of an electric squib partially in section.

The squib is shown in generally conventional form. Drawn aluminum closed end shell 11 contains in its lower or closed portion an initiating charge 13 of black powder. Shell 11 is supplied with a bead 15 near its top or open end. Leg wires 17 and 19 for application to a source of current extend through sealing compositions 21 and 22, made of sulphur and asphaltic waterproofing composition respectively, which hold them in

2

place and seal the end of shell 11. Sealing composition 21 is held in place by bead 15. Inside shell 11 above charge 13 and connected to leg wires 17 and 19 is located electric fuse-head assembly 23. In operation leg wires 17 and 19 are connected to a source of electric current which fires fusehead 23 which in turn ignites charge 13. Charge 13 then bursts shell 11 and fires an explosive to be initiated.

10 Numerous modifications of the electric initiator shown are, of course, possible as is well known in the art. For example, the shell may be made of materials other than aluminum. Initiating charge 13 which is represented in the drawing as 15 a single charge of black powder may, instead, be in the form of a plurality of separate charges of the same or a different composition. Seals 21 and 22 may be of any suitable compositions, and instead of a double seal as shown in the drawing 20 a single or any plurality of seals may be used. In addition to, or instead of, bead 15, the shell may be supplied with other plug fastening means, such as crimps, internal knurls, etc. In place of fusehead 23, other suitable igniting means, such 25 as bridge wires or spark gaps, with such flash compositions as may be desirable, may be employed.

As has been indicated above, it is usually desired that the initiating force be directed out 30 through the initiator shell. Various methods of assuring this action have been proposed in the prior art. For example, one proposal has been to score the initiator shell so as to weaken it at the scored places and thereby make it easier to 35 rupture. This method, while operative, is difficult to perform in that it is quite a problem to control the depth of the scores and to insure that they are sufficient to provide adequate rupturability but do not puncture the shell completely.

40 A second method, useful for squibs, that has been suggested is locating a small portion of detonating explosive in the bottom of the squib near the initiating charge and adjacent the shell. The detonating explosive opens a hole in the shell for 45 the escape of the burning discharge from the squib. This method is clumsy, adds considerably to the difficulty of manufacturing squibs, and makes squibs more dangerous because of the detonating explosive which must be included in 50 them. A third method also applicable to squibs is to employ a heat-producing charge which melts the shell wall. This method, of course, has the disadvantage that a special charge must be employed.

55 According to the present invention, an initiator

is provided which may employ ordinary and conventional charges, but which at the same time has a shell readily rupturable at any desired point, by providing a limited area of the shell relatively and materially softer than remaining areas of the shell. In a preferred embodiment of the invention, a local portion of the shell is annealed to a softened condition while remaining portions are left hard. In this way, a place of easy rupturability is provided through which the initiating force may be directed.

For example, drawn shell 11 of the initiator shown in the drawing is, before being charged with explosive, annealed adjacent the portion to be charged, making that portion soft so that the squib flame will burst the shell and discharge therethrough, while the top portion of the shell is left hard and strong so as to provide an efficient grip on the sealing plug and prevent its blowing out with consequent dissipation of the initiating force in the wrong direction.

The annealing operation may be conducted in any convenient manner. The temperature and time necessary depend upon the particular material involved and the amount of working which it has undergone while being shaped. They will also, of course, further depend upon the particular softness which it is desired to achieve. In general, the higher the temperature, the shorter the time needed. For any particular job, conditions for annealing are easily found. When annealing, care should be maintained to insure that the portion of the shell which it is desired to keep hard does not become so heated by conduction that it is also annealed. While such a portion may be externally cooled, it is often sufficient that the annealing be performed rapidly, for in that way it is possible that the desired portions may be softened before remaining portions become heated. With drawn aluminum shells, which have been found especially adaptable to the present invention, the annealing operation may be carried out by simple heating of the portion of the shell, which it is desired to soften, in a Bunsen flame for about a second. Other material, as indicated above, requires heating to a different temperature and/or time, and may also require quenching procedures. Gilding metal is an example of a metal which requires a higher temperature of anneal. Instead of metals, plastic materials which have been locally softened may be used in some embodiments of this invention. For example, vinylidene chloride polymers, which may be work-hardened, have many of the properties of metals and may be formed and annealed to produce initiator shells according to the present invention.

Desirable directed rupturing of aluminum electric squib shells and adequate prevention of plug blowouts has been obtained when the top portions of the aluminum shells have been kept at a hardness as low as 8 as determined by means of a Shore scleroscope having a magnifier hammer, and when the softened portions have a hardness as high as 5. The parts of the shells extending about one-quarter inch down from their tops are considered to be top portions. If the hardness of the top portions of the shells is permitted to get lower than about 8 and the hardness of the softened portions is greater than about 5, plug blowouts occur under severe conditions of operation.

It is possible by the use of more concentrated flame playing on a small area to obtain softened portions having a hardness considerably below 5, while retaining the desired hardness at the tops.

In fact, better results have been obtained when the softened portions show hardnesses of about 2½ to 3. Usually, it is desirable that hardnesses of much below 2 be avoided as attempts to lower the hardness much below this figure have often resulted in undue weakening or actual burning through of the shells.

It has been found desirable to locate the softened portion of the shell at about the top level of the explosive charge. If the soft portion is placed much lower on the shell, plug blowouts will sometimes occur under difficult conditions of operation. Apparently, in such cases, force sufficient to blow the plug is obtained before sufficient explosive action at the point of softening takes place.

The invention will be more specifically illustrated by the following examples. In each of these examples, drawn aluminum shells, each of which was about 2¼ in. long, about 0.275 in. in outside diameter, and about 0.006 in. in wall thickness, were annealed by passing the shells in an inverted position past two gas-oxygen torches simultaneously directed horizontally against them. The torches were fed by propane gas from a cylinder, and oxygen at a pressure of about 2 lbs. per sq. in. The shells were moved intermittently so that each was acted on by the flame for a period of about four-fifths second. Immediately after passing through the flame, a jet of air was directed against the tops of the shells and the shells were permitted to cool. A number of each batch were spread open, flattened, and their hardnesses measured in different portions with a Shore scleroscope, using the magnifier hammer. Other of the shells were charged and sealed to prepare electric squibs in the conventional form heretofore described. Each squib contained a charge of black powder, reaching about one inch from the bottom of the shell.

#### Example 1

A number of shells were annealed with the torches adjusted so that each shell had a soft band about 5/8 in. wide, the center of which was about 1 in. from the bottom of the shell. The soft band had a hardness ranging from 2 to 3. The hardness of these same shells taken near the top of the shell was from 8 to 10. 195 shells of this number were made up into electric squibs and placed in a cooling chest where they were cooled to -60° F. After being removed from the chest and promptly fired, none of these shells showed blowouts and none showed loose plugs. The temperature of -60° F. was selected for cooling because it represents a particularly severe test condition for electric squibs.

#### Example 2

60 100 squibs prepared from shells unannealed, but otherwise similar to those of Example 1, were similarly fired after cooling to -60° F. Of these, the plugs of 25 blew out.

#### Example 3

A number of shells were prepared and tested as described above, but the torches were adjusted so that the softened band was narrowed to about 5/16 in. The center of this band was again located about 1 in. from the bottom of the shell. The hardness of the soft band was 2 to 3 and the hardness near the top was 8 to 10. When 23 squibs prepared from these shells were fired after cooling to -60° F. there was no evidence of plug blowout or plug loosening.

*Example 4*

A number of shells were again prepared, but this time only one flame was used and it was adjusted so that the annealed portion was cut down to a spot about  $\frac{1}{4}$  in. in diameter. This spot was located about 1 in. from the bottom of the shell. The annealed portion showed a hardness of 2 to 4, and the top portion showed a hardness of 8 to 10. 25 squibs prepared from these shells were fired after cooling to  $-60^{\circ}$  F., and no blowouts or plug loosenings occurred. It was noted that a number of the shells on firing opened only in the area represented by the softened spot. When soft portions of greater area were prepared, the shells usually opened in about a  $\frac{1}{2}$  in. band almost completely around the circumference.

*Example 5*

Shells were prepared as in Example 4, but this time the annealed spot was softened to a hardness of only 5 to 6. The top portion again showed a hardness of about 8 to 10. Out of 21 squibs prepared with these shells and fired after cooling to  $-60^{\circ}$  F., 5 plugs blew out and 3 were loose.

*Example 6*

A number of shells were annealed so as to produce a soft  $\frac{1}{2}$  in. band having a hardness of about 2-3, while the top portions of the shells showed hardnesses of about 8-10. In this case, however, the  $\frac{1}{2}$  in. softened band was located at the bottom of the shell. Of fifty squibs prepared from these shells and fired after cooling to  $-60^{\circ}$  F., 3 plugs blew out.

*Example 7*

A number of shells were annealed so as to produce a  $\frac{5}{8}$  in. band ending 1 in. from the bottom of the shell. The softened bands showed a hardness of about 2-3, while the top portion of the shells maintained a hardness of about 8-10. Of 50 squibs prepared from such shells, one plug blew out on firing after cooling to  $-60^{\circ}$  F.

The invention is not to be considered as necessarily being limited to the specific embodiments disclosed. For instance, it is not necessary that the annealing operation be performed by means of a hot flame or that the cooling operation when employed be performed by an air blast. Other sources of heat as electric heating, for example, may be employed, and also any suitable cooling media may be employed if desired.

Also, the invention need not be restricted to aluminum shells or squibs, but is applicable in its

broader aspects wherever directed initiation is desired, and it is also applicable to other types of initiators, such as detonators, and to other types of shells.

5 The invention will further be found applicable to initiator shells which have been given a partial overall anneal. It is necessary only that there be hardness which can be locally annealed.

In the claims where hardnesses are mentioned, 10 it is to be understood that they are Shore sclerometer hardnesses measured with the magnifler hammer and determined on shells which have been opened and unrolled into a flattened condition.

15 What is claimed is:

1. An electric squib which comprises a drawn aluminum shell having a closed bottom, an explosive charge in said shell, a portion of said shell adjacent the top portion of said charge being annealed to a soft condition, and a sealing composition closing the top of said shell.

2. An electric squib according to claim 1 in which the top portion of the shell has a hardness no less than about 8 and in which the soft portion has a hardness no greater than 5.

25 3. An electric explosion initiator which comprises a drawn metal shell having a closed bottom, an explosive charge in said shell, and a seal closing the top of said shell; a portion of said shell adjacent said explosive charge being annealed to a soft condition so as to provide a place of easy rupturability through which the initiating force may be directed.

35

WILLIAM F. REAGER.

## REFERENCES CITED

The following references are of record in the file of this patent:

## 40 UNITED STATES PATENTS

| Number       | Name           | Date           |
|--------------|----------------|----------------|
| Re. 18,837   | Rolland        | May 23, 1933   |
| 411,206      | Smith          | Sept. 17, 1889 |
| 45 2,007,959 | Babbitt et al. | July 16, 1935  |
| 2,112,974    | Noddin         | Apr. 5, 1938   |
| 2,220,652    | Irmann         | Nov. 5, 1940   |
| 2,325,079    | Soderholm      | July 27, 1943  |

## 50 FOREIGN PATENTS

| Number | Country       | Date |
|--------|---------------|------|
| 878    | Great Britain | 1913 |
| 15,958 | Great Britain | 1885 |

55